

Nov. 23, 1965

K. SEIDLER

3,218,832

PHOTOFFLASH LAMP AND METHOD

Filed Sept. 26, 1963



Inventor:  
Karl Seidler  
by Henry T. Olsen  
His Attorney

## 1

3,218,832

## PHOTOFFLASH LAMP AND METHOD

Karl Seidler, Augsburg, Germany, assignor to Patent-Treuhand-Gesellschaft fur elektrische Glühlampen m.b.H.

Filed Sept. 26, 1963, Ser. No. 311,751  
Claims priority, application Germany, Nov. 9, 1962,  
P 30,539

2 Claims. (Cl. 67—31)

The present invention relates to photoflash lamps having a glass envelope and a filling of combustible material and oxygen and more particularly to a splinterproof protective coating therefor.

When a lamp is flashed, an instantaneous peak pressure is created in the envelope and the glass envelope is brought to high temperature for a short time. Because of the high superpressure at the moment of flashing, the glass envelope tends to break into pieces. In order to prevent this latter or to hold together the glass splinters, the outer or inner or both of the surfaces of the bulb are provided with a splinterproof coating of lacquer.

In the case of well known photoflash lamps wherein the pressure of the oxygen filling does not much exceed atmospheric pressure a splinterproof coating of cellulose acetate butyrate has been used. The lamp bulb was coated by dipping it once into a dipping bath consisting of a solution of cellulose acetate butyrate in a solvent and in most cases containing a softener.

In the case of miniature photoflash lamps developed recently and having an oxygen pressure of much more than one atmosphere such a single lacquering with cellulose acetate butyrate did not prove satisfactory. Because of a very high peak pressure and high peak temperature many of the lamps burst and all flashed lamps show a considerable change in the lacquer coating, such as molten places and formation of blisters. Also, at the moment of flashing there was an intense development of smoke by the lacquer coating which has a very bad effect on the reflector surface of the flash device and which had a very strong smell associated therewith. Because of this a lacquering of cellulose acetate has been used in miniature photoflash lamps. Sufficient high strength may, however, be obtained with this material only by repeated lacquering, which repeated lacquering increases the cost of manufacture. Furthermore, a splinterproof coating made by repeated lacquering with cellulose acetate does not remain unchanged when flashed, but still shows formation of blisters, molten places, and development of smoke.

It is an object of the present invention to provide a splinterproof lacquer coating which has, in the case of miniature photoflash lamps with high filling pressure, sufficient protective effect even as single coating and does not show any formation of blisters, molten places or development of smoke.

Therefore, in accordance with the present invention there is provided a photoflash lamp having a glass envelope, a filling of combustible material and oxygen at a pressure exceeding one atmosphere and a splinterproof lacquer coating which consists essentially of cellulose propionate.

The accompanying drawing shows a miniature photoflash lamp with an oxygen pressure exceeding one atmos-

## 2

phere and coated with a splinterproof lacquer coating in accordance with the invention.

The envelope 1 of the miniature photoflash lamp is filled with combustible material 2, e.g. with shredded zirconium foils in an oxygen atmosphere the pressure of which is higher than one atmosphere. By means of the igniting device 3 which is in well known manner actuated by means of the contacts 4 being taken outwards through the seal, combustion of the filling is brought about and, thereby, the light emission. The envelope is provided with a protective coating 5 consisting of a lacquer according to the invention which consists essentially of cellulose propionate.

Generally, the coating is applied by dipping into a solution of cellulose propionate. The dipping solution contains, preferably, beside a solvent also an addition of up to 10% by weight of a softener. Dibutyl sebacate has proved to be especially good as the softener.

A dipping lacquer for instance is composed of 80% by weight of a solvent, 18% by weight of cellulose propionate and 2% by weight of dibutyl sebacate.

The solvent for the cellulose propionate and the softener includes preferably 3 parts of a low boiling, i.e., a boiling temperature from 75–77° C., material such as ethyl acetate, methanol and/or ethanol, 2 parts of an intermediate boiling, i.e., a boiling temperature from 138–152° C., material such as methyl glycol acetate and 1 part of a high boiling, i.e., a boiling temperature from 160–170° C., material such as diacetone alcohol.

Thus, a very suitable dipping lacquer for obtaining, in a single dipping, sufficient splinterproof protection of the miniature photoflash lamps without any formation of blisters or any development of smoke when these lamps are flashed consists of

30% by weight ethyl acetate  
14% by weight methanol  
6% by weight ethanol  
20% by weight methyl glycol acetate  
10% by weight diacetone alcohol  
18% by weight cellulose propionate  
2% by weight softener dibutyl sebacate.

The percentages of the different solvents are, suitably, chosen in such a manner that there is obtained preferably a viscosity of 200 sec./22° C. Ford-cup 8 mm.

For lamps having an oxygen pressure of 2 to 4 atmosphere a single dipping with the splinterproof lacquer described in the present invention is sufficient whereas two dippings are necessary if cellulose acetate is used. In case of even higher filling pressures of the lamps two dippings with a lacquer of cellulose propionate are sufficient whereas, hitherto, in case of cellulose acetate 4 dippings have been necessary.

In order to adapt the light emission of the photoflash lamps to sensitivity of, e.g., color films, a suitable coloring substance may also be added, if desired, to the dipping lacquer.

What is claimed as new and desired to be secured by Letters Patent of the United States is:

1. A photoflash lamp comprising a glass envelope, a filling in said envelope of combustible material and oxygen at a pressure exceeding one atmosphere, and a splinterproof protective coating on the exterior surface of the glass envelope consisting essentially of cellulose propionate.

2. A photoflash lamp comprising a glass envelope, a filling in said envelope of combustible material and oxygen at a pressure exceeding one atmosphere, and a splinterproof protective coating on the exterior surface of the glass envelope consisting essentially of cellulose propionate and a small amount of dibutyl sebacate plasticizer. 5

2,868,670 1/1959 Van Laar et al. ----- 67—31  
2,927,036 3/1960 Seaver ----- 106—181 X  
3,022,653 2/1962 Baird ----- 67—31  
3,068,112 12/1962 Caldwell et al. ----- 106—181 X

## OTHER REFERENCES

Publication: Cellulosics, by W. D. Paist, 1958, Reinhold Publ. Corp., Chapman and Hall Ltd., London, TP 986 A2, p. 33, pps. 34—37 relied on.

EDWARD J. MICHAEL, *Primary Examiner.*

## References Cited by the Examiner

## UNITED STATES PATENTS

2,510,177 6/1950 Horback ----- 106—181 10  
2,673,162 3/1954 Williams et al. ----- 106—181